

# United States Patent

Merli et al.

[15] 3,655,391

[45] Apr. 11, 1972

[54] **AZODICARBONAMIDE FOG INHIBITORS**

[72] Inventors: **Paoli Merli**, Condominio Isonzo-Via Colombo, Pordenone; **Luigi Valbusa**, Via Gramsci, Ferrania, Savona, both of Italy

[22] Filed: **Oct. 23, 1969**

[21] Appl. No.: **868,908**

**Related U.S. Application Data**

[63] Continuation-in-part of Ser. No. 856,485, Sept. 9, 1969.

[30] **Foreign Application Priority Data**

May 16, 1969 Italy ..... 37,118 A/69  
Aug. 1, 1969 Italy ..... 39,154 A/69  
Sept. 9, 1969 Italy ..... 39,648 A/69

[52] U.S. Cl. .... **96/109, 96/66.5, 260/192,**  
260/553

[51] Int. Cl. .... **C07c 107/02, G03c 1/34**

[58] Field of Search. .... **96/109, 66.5, 67, 68, 95;**  
260/553, 554, 192

[56]

**References Cited**

**UNITED STATES PATENTS**

|           |        |                 |           |
|-----------|--------|-----------------|-----------|
| 2,988,545 | 6/1961 | Hill.....       | 260/192   |
| 3,100,704 | 8/1963 | Coles.....      | 96/109 X  |
| 3,128,187 | 4/1964 | Sagal.....      | 96/109    |
| 3,134,764 | 5/1964 | Blout.....      | 260/192 X |
| 3,396,023 | 8/1968 | Rees.....       | 96/67     |
| 3,396,028 | 8/1968 | Humphlett.....  | 96/109    |
| 3,499,761 | 3/1970 | Binghamton..... | 96/66.5   |
| 3,505,308 | 4/1970 | Smith.....      | 260/192   |

Primary Examiner—John T. Gookasian

Assistant Examiner—M. E. McCamish

Attorney—Kinney, Alexander, Sell, Steldt and DeLaHunt

[57]

**ABSTRACT**

Azodicarbonamides, preferably having the general formula



wherein R<sub>1</sub>, R<sub>2</sub>, R<sub>3</sub> and R<sub>4</sub> individually are hydrogen, alkyl, aryl, or heterocyclic groups, or wherein the pairs of groups R<sub>1</sub>—R<sub>2</sub> or R<sub>3</sub>—R<sub>4</sub> represent atoms necessary to complete a heterocyclic ring, are effective fog-inhibitors for silver halide photographic emulsions.

**11 Claims, No Drawings**

## AZODICARBONAMIDE FOG INHIBITORS

This application is a continuation-in-part of pending United States application Ser. No. 856,485, filed Sept. 9, 1969.

This invention relates to compounds useful as anti-fog, anti-stain, and stabilizing agents for silver halide photographic emulsions. More particularly, this invention relates to silver halide photographic emulsions containing such compounds and to photographic elements prepared from such emulsions.

The silver metal which appears in unexposed areas of a silver halide photographic element upon development is commonly referred to as "fog". Fog may often be traced to the action of certain emulsion components, to the composition or nature of the developer, to atmospheric oxidation, to aging, etc. The type of packaging used for photographic film may influence fog formation, as may the type of film support upon which a silver halide emulsion is coated. For example, a polyester supporting film is more likely to contribute to the presence of fog in an overlying emulsion layer than in a cellulose ester supporting film. The aging of silver halide emulsions at high temperatures and high humidities generally favors the formation of fog.

Although fog generally appears as a uniform darkening of an emulsion layer in a photographic element, such layers also often exhibit small areas in which the fogging is much greater or less than that of the surrounding areas. Such small areas commonly are referred to as "sensitization" or "desensitization" spots, or more simply, as "black spots" and "white spots". These spots have often been traced to the presence in the emulsion layer (or in a layer adjacent thereto) of metal particles such as particles of iron, copper, tin, etc., or compounds thereof. Such particles in turn are generally traceable to the type of supporting film utilized (e.g., polyester) or to the general environment in which the photographic material had been prepared or utilized.

Reduction or elimination of both fog and the above-described "spotting" in silver halide emulsions is greatly desired.

It has now been found that fog and "spotting" (both of which are hereinafter referred to collectively as "fog") in a silver halide emulsion can be greatly inhibited by employing as a fog inhibitor an azodicarbonamide, preferably a compound of the general formula



wherein  $\text{R}_1$ ,  $\text{R}_2$ ,  $\text{R}_3$  and  $\text{R}_4$  individually are hydrogen or an alkyl, aryl, or heterocyclic group, or wherein pairs of groups  $\text{R}_1 - \text{R}_2$  or  $\text{R}_3 - \text{R}_4$  represent atoms necessary to complete a heterocyclic ring. "Alkyl" and "aryl" as used herein include substituted alkyl (e.g., alkoxyalkyl, hydroxyalkyl, aralkyl, etc.) and substituted aryl (e.g., alkaryl, arkoxyaryl, etc.) groups.

Accordingly, the invention in one aspect relates to a silver halide emulsion having contacted therewith an azodicarbonamide compound. In another aspect the invention relates to a photographic element having a silver halide emulsion layer and having an azodicarbonamide compound in fog-inhibiting association therewith (e.g., in a layer adjacent the emulsion layer). In another aspect the invention relates to a method for inhibiting fog in a silver halide photographic emulsion comprising contacting the emulsion with an azodicarbonamide. The invention in a further aspect relates to certain novel azodicarbonamide compounds capable of inhibiting fog in silver halide emulsions and having the formula



wherein  $\text{R}_5$ ,  $\text{R}_6$ ,  $\text{R}_7$  and  $\text{R}_8$  may be hydrogen and wherein at least one of  $\text{R}_5$ ,  $\text{R}_6$ ,  $\text{R}_7$  and  $\text{R}_8$  is an alkoxyalkyl, alkoxyaryl, hydroxyalkyl, haloaryl, allyl, heterocyclic or heterocyclic alkyl group.

5 Azodicarbonamide compounds as a class have been found capable of inhibiting the formation of fog in a silver halide photographic emulsion when contacted therewith. By "contacted" as used herein is meant that the azodicarbonamide is placed in fog-inhibiting association with the emulsion. For example, the azodicarbonamide may be incorporated within the emulsion, or in an adjacent layer, or in various photographic processing (e.g., developer) baths or the like. It has been found that the selection of the  $\text{R}_1 - \text{R}_4$  groups in the above-described formula does not greatly vary the capacity of the compounds to inhibit fog. Examples of compounds representative of the various classes of substituted azodicarbonamides are as follows:

## EXAMPLE 1 - N,N' - DIMETHYL-AZODICARBONAMIDE

10 17.4 g. (0.1 mol) of azodicarboxylic acid ethyl ester were dissolved in 100 ml. of diethyl ether, and to this solution 6.5 g. (0.21 mol) of methylamine in a 33 percent ethanol solution were added. The reaction occurred at 32.0° F. (0° C.) and was immediate. After washing with diethyl ether, 9.3 g. of raw material were recovered in the form of an orange-colored powder, from which 7.79 of long orange-colored needles having a melting point of 336.2° F. (169° C.) were obtained by crystallization from ethyl acetate.

|           |    | Calculated | Found |
|-----------|----|------------|-------|
| Analysis: | C% | 33.40      | 33.46 |
|           | H% | 5.56       | 5.66  |
|           | N% | 38.87      | 38.72 |

## EXAMPLE 2 - N,N' - DIETHYL-AZODICARBONAMIDE

20 Azodicarboxylic acid ethyl ester (26.1 g.) were dissolved in 200 ml. of diethyl ether and to this solution 13.5 of ethylamine in a 33 percent ethanol solution were added, the temperature being maintained below 68.0° F. (20° C.). The product was filtered, washed with diethyl ether and dried under vacuum. Yellow crystals (19 g.) having a melting point of 273.2° - 275.0° F. (134° - 135° C.) were recovered.

|           |    | Calculated | Found |
|-----------|----|------------|-------|
| Analysis: | C% | 41.90      | 41.97 |
|           | H% | 6.98       | 7.02  |
|           | N% | 32.56      | 32.41 |

## EXAMPLE 3 - N,N' - DIPROPYL-AZODICARBONAMIDE

30 To 17.4 g. (0.1 mol) of azodicarboxylic acid ethyl ester dissolved in 100 ml. of diethyl ether were added 12.4 g. (0.21 mol.) of propyl amine in 50 ml. of diethyl ether.

The reaction, carried out with external cooling at 32.0° F. (0° C.), was immediate and moderately exothermic.

35 The product was collected and washed with diethyl ether to provide 13 g. of an orange-colored powder. By crystallization from 500 ml. of ethyl acetate, 10 g. of small, orange-colored needles having a melting point of 305.6° F. (152° C.) were obtained.

|           |    | Calculated | Found |
|-----------|----|------------|-------|
| Analysis% | C% | 48.00      | 47.81 |
|           | H% | 8.02       | 8.13  |
|           | N% | 28.05      | 28.06 |

## EXAMPLE 4 - N,N' - DI - 2 - METHOXYETHYL-AZODICARBONAMIDE

7.8 g (0.1 mol.) of 2-methoxyethylamine dissolved in 50 ml. of diethyl ether were added to a solution of 8.7 g (0.05 mol.) of azodicarboxylic acid ethyl ester in 100 ml. of diethyl ether. The reaction was carried out at 32.0° F. (0° C.). 65. g of product were recovered, from which, by crystallization from 120 ml. of ethyl acetate, 4.5 g of small, orange-colored needles having a melting point of 222.8° F. (106° C.) were obtained.

boxylic acid ethyl ester in 100 ml. of diethyl ether at 32° F. (0° C.).

The solid which separated was washed with diethyl ether to provide 17.5 g of product. Crystallization from ethyl acetate yielded 12.5 g of small, orange-colored needles having a melting point of 217.4° F. (103° C.).

|    |                          | Calculated             | Found                  |
|----|--------------------------|------------------------|------------------------|
| 10 | Analysis: C%<br>H%<br>N% | 46.20<br>7.69<br>21.57 | 45.68<br>7.72<br>21.66 |

|                          | Calculated             | Found                  |
|--------------------------|------------------------|------------------------|
| Analysis: C%<br>H%<br>N% | 41.30<br>6.90<br>24.15 | 41.28<br>7.11<br>24.41 |

## EXAMPLE 5 - N,N' - DALLY-AZODICARBONAMIDE

Allylamine (12.0 g; 0.21 mol) in three times its volume of diethyl ether, was added to 17.4 g (0.1 mol.) of azodicarboxylic acid ethyl ester in 5 times its volume of diethyl ether at 32.0° F. (0° C.). The amide (14 g) separated out almost immediately. By crystallization from 300 mol. of ethyl acetate, 9.5 g of small, orange-colored needles having a melting point of 291.2° F. (144.0° C.) were recovered.

|                          | Calculated             | Found                  |
|--------------------------|------------------------|------------------------|
| Analysis: C%<br>H%<br>N% | 48.90<br>6.16<br>28.55 | 49.07<br>6.28<br>28.77 |

## EXAMPLE 6 - N,N' - DIISOPROPYL-AZODICARBONAMIDE

To 17.4 g. (0.1 mol.) of azodicarboxylic acid ethyl ester in 100 ml. of diethyl ether were added 12.4 g. (0.21 mol.) of isopropylamine in 50 ml. of diethyl ether at 32.0° F. (0° C.). A yellow-colored product (5.3 g.) separated out from which, by crystallization from ethyl acetate, 2.5 g. of small, pale, orange-colored needles were obtained. By evaporation of the mother liquors, another crop of product having a melting point of 316.4° F. (158° C.) separated out, yielding 4.3 g. of total product.

|                          | Calculated             | Found                  |
|--------------------------|------------------------|------------------------|
| Analysis: C%<br>H%<br>N% | 48.00<br>8.07<br>28.05 | 47.80<br>8.10<br>28.15 |

## EXAMPLE 7 - N,N' - DIBUTYL-AZODICARBONAMIDE

15 g. (0.21 mol.) of n-butylamine dissolved in 50 ml. of diethyl ether, and 17.4 g. (0.1 mol.) of azodicarboxylic acid ethyl ester, in 100 ml. of diethyl ether, were mixed at 32.0° F. (0° C.). The solid which separated out was washed with diethyl ether and purified by crystallization from ethyl acetate. 12 g of small orange-colored needles having a melting point of 318.2° F. (159° C.) were recovered.

|                          | Calculated             | Found                  |
|--------------------------|------------------------|------------------------|
| Analysis: C%<br>H%<br>N% | 52.90<br>8.78<br>24.52 | 52.86<br>8.74<br>24.53 |

## EXAMPLE 8 - N,N' - DI - 2 - ETHOXYETHYL-AZODICARBONAMIDE

18 g (0.21 mol) of 2-ethoxyethylamine in 50 ml. of diethyl ether were added dropwise to 17.4 g (0.1 mol) of azodicar-

## EXAMPLE 9 - N,N' - BIS-[ (2-PYRIDYL)METHYL] - AZODICARBONAMIDE



25 To 17.4 g (0.1 mol) of azodicarboxylic acid ethyl ester in 50 ml. of diethyl ether were added 21.8 g (0.21 mol) of amino-2-picoline in 25 ml. of diethyl ether at 32° F. (0° C.). The reaction was immediate and the amide which separated out at once was washed with diethyl ether to provide 23 g of a pink-colored powder. By crystallization from 600 ml. of methanol and concentration of the mother liquors, 10 g of orange yellow crystals having a melting point of 334.4° F. (168° C.) were obtained

|                          | Calculated             | Found                  |
|--------------------------|------------------------|------------------------|
| Analysis: C%<br>H%<br>N% | 56.35<br>4.70<br>28.15 | 55.87<br>4.86<br>27.90 |

## EXAMPLE 10 - N,N' - DI - (3-PYRIDYLETHYL) - AZODICARBONAMIDE



50 To 9.5 g of azodicarboxylic acid ethyl ester in 100 ml. of diethyl ether, 10.8 g of 2-amino-3-picoline in 50 ml. of diethyl ether were added at a temperature lower than 20° C. The reaction was isothermal and the solid amide separated out at once.

55 By crystallization from methanol, orange yellow crystals having a melting point of 164°-162° C. were obtained.

|                          | Calculated             | Found                  |
|--------------------------|------------------------|------------------------|
| Analysis: C%<br>H%<br>N% | 56.35<br>4.70<br>28.15 | 56.38<br>5.08<br>28.16 |

## EXAMPLE 11 - N,N' - DI - (4-PYRIDYL METHYL) - AZODICARBONAMIDE



To 9.5 g of azodicarboxylic acid ethylester in 100 ml. of diethylether, 10.8 g of -amino-4-picoline in 50 ml. of ether were added at a temperature lower than 20° C. The reaction

was isothermal and the solid amide separated out at once, then it was washed with diethylether. By crystallization from ethanol small orange crystals having a melting point of 157°-159° C. were obtained.

|              | Calculated | Found |
|--------------|------------|-------|
| Analysis: C% | 56.25      | 56.31 |
| H%           | 4.7        | 4.99  |
| N%           | 28.15      | 27.88 |

#### EXAMPLE 12 - N,N' - BIS (2-HYDROXYETHYL) - AZODICARBONAMIDE

To 17.4 g (0.1 mol) of azodicarboxylic acid ethyl ester, dissolved in 100 ml. of diethyl ether were added 12.4 g (0.21 mol) of ethanalamine dissolved in a mixture of 25 ml. of 5 ethanol and 25 ml. of diethyl ether at 32° F (0° C).

The reaction occurred immediately and the amide (17 g) separated out and was crystallized from 350 ml. of methanol 9.5 g of small orange-colored needles having a melting point of 285.8° F (141° C) were recovered.

|              | Calculated | Found |
|--------------|------------|-------|
| Analysis: C% | 35.83      | 35.35 |
| H%           | 5.97       | 6.00  |
| N%           | 27.88      | 27.28 |

#### EXAMPLE 13 - N,N' - BIS (3-HYDROXYPROPYL) - AZODICARBONAMIDE

To 17.4 g (0.1 mol) of azodicarboxylic acid ethyl ester dissolved in 100 ml. of diethyl ether were added 15.5 g (0.21 mol) of 3-propanolamine dissolved in a mixture of 25 ml. of ethanol and 25 ml. of diethyl ether at 32.0° F (0° C). The reaction occurred immediately and the amide (21 g) separated out and was purified by crystallization from 150 ml. of ethanol. 16.5 g of small, orange-colored needles having a melting point of 284.0° F. (140° C) were recovered.

|              | Calculated | Found |
|--------------|------------|-------|
| Analysis: C% | 41.30      | 41.23 |
| H%           | 6.93       | 6.99  |
| N%           | 24.10      | 23.87 |

#### EXAMPLE 14 - N,N' - DIPHENYL - AZODICARBONAMIDE

To 8.1 g of hydrazodicarbonamide (prepared by pyrolysis of 4-phenylsemicarbazide suspended in 200 ml. of pyridine was added a solution of 5.5 g of N-bromo-succinimide dissolved in 100 ml. of pyridine at a temperature of 95.0° F (35.0° C). The solid dissolved slowly and the solution became dark red in color. After about two hours, the solution was vacuum filtered and the filtrate was quickly poured into two liters of ice water. A fluffy red-colored solid separated out which was then filtered, washed with water and crystallized from 150 ml. of hot ethyl acetate. Red colored plates having a melting point of 347.0° - 350.6° F (175° - 177° C) were obtained.

|              | Calculated | Found |
|--------------|------------|-------|
| Analysis: C% | 62.70      | 62.80 |
| H%           | 4.47       | 4.69  |
| N%           | 20.85      | 20.74 |

#### EXAMPLE 15 - N,N' - DI - M-CHLOROPHENYL - AZODICARBONAMIDE

To 92.8 g of nitrochlorophenyl - 4 - semicarbazide dissolved in 1200 ml. of ethanol, 25.4 g of iodine were added portion

wise at the boil. The mass was allowed to boil for half an hour and was filtered hot. The resulting whitish solid (hydrazo compound) was washed with hot water and dried under vacuum at a temperature of 132.8° F (56° C). To 6.8 g of the N,N'-di-5-chlorophenylhydrazo dicarbonamide, suspended in 100 ml. of pyridine was added dropwise at 45° - 50° C 7.6 g of N-bromo-succinimide in 150 ml. of pyridine. The resulting solution was poured into 1.5 liters of ice water and the orange-red colored precipitate which was obtained was washed with water and crystallized from 200 ml. of hot ethyl acetate.

Extremely thin, orange red-colored, needles were obtained which decomposed at 341.6° - 345.2° F (172° - 174° C).

|              | Calculated | Found |
|--------------|------------|-------|
| Analysis: C% | 49.80      | 48.94 |
| H%           | 2.97       | 2.96  |
| N%           | 16.62      | 16.67 |

#### EXAMPLE 16 - N,N' - DI - $\rho$ - TOLYL - AZODICARBONAMIDE

To 14.9 g of N,N' - di -  $\rho$  - tolyl hydrazodicarbon-amide (obtained by pyrolysis of 4-p-tolyl-semicarbazide) suspended in 300 ml. of pyridine, 17.8 g of N-bromo-succinimide dissolved in 200 ml. of pyridine were added dropwise at a temperature of 158.0° F (70° C). The resulting solution was poured into ice water, and the orange-red precipitate which formed was filtered, washed, dried, under vacuum at room temperature, and was crystallized from hot ethyl acetate. The resulting compound, in the form of small deeply orange-red-colored needles, decomposed at 341.6° - 347.0° F (172° - 175° C).

|              | Calculated | Found |
|--------------|------------|-------|
| Analysis: C% | 64.76      | 65.19 |
| H%           | 5.40       | 5.72  |
| N%           | 18.80      | 18.26 |

#### EXAMPLE 17 - N,N' - DI - $\rho$ - METHOXYPHENYL - AZODICARBONAMIDE

To 6.6 g of hydrazodicarbonamide (obtained by pyrolysis of paramethoxyphenyl-4-semicarbazide) suspended in 150 ml. of pyridine was added dropwise 7.2 g of N-bromo-succinimide in 100 ml. of pyridine. The resulting solution was poured into ice water, and the dark red precipitate which was formed was washed with water, dried under vacuum, and crystallized from hot ethyl acetate. Dark-red colored needles, melting at 336.2° - 350.6° F (169° - 177° C) were obtained.

|              | Calculated | Found |
|--------------|------------|-------|
| Analysis: C% | 58.50      | 58.50 |
| H%           | 4.78       | 4.92  |
| N%           | 17.06      | 16.92 |

#### EXAMPLE 18 - N,N' - DI - ( $\alpha$ -PYRIDYL) - AZODICARBONAMIDE

Equimolecular amounts of  $\alpha$  -amino-pyridine and diethylazo-dicarboxylate was reacted, in alcohol solution, at a temperature not exceeding 59.0° F (15° C). After the completion of the reaction, the mass was allowed to stand undisturbed overnight and the product which separated out was collected by suction. A dark yellow powder melting at 350.6° - 354.2° F (177° - 179° C.) was obtained.

#### EXAMPLE 19 - N,N' - DI - ( $\beta$ -PYRIDYL) - AZODICARBONAMIDE

Equimolecular amounts of  $\beta$  -amino-pyridine and diethyl azodicarboxylate were reacted, in alcohol solution, at 50.0° - 59.0° F (10° - 15° C.). After the completion of the reaction,

the mass was allowed to stand undisturbed overnight and the product which separated out was collected by suction. By repeatedly extracting the product with hot alcohol and concentrating the liquid under vacuum, needle-like crystals were obtained having an M.p. of 327.2° F (164° C.).

**EXAMPLE 20 - N,N' - DI - (γ -PYRIDYL)  
AZODICARBONAMIDE**

Equimolecular amounts of γ -amino-pyridine and diethylazo-dicarboxylate were reacted in pyridine at 59.0° F (15° C.). The reaction was allowed to go to completion overnight at room temperature.

The reaction product was a crystalline, yellow-colored solid melting at 352.4° - 357.8° F (178° - 181° C.).

**EXAMPLE 21 - N,N' - DI - (γ -FURYL)  
AZODICARBONAMIDE**

2.5 g of N,N' -γ -furyl-hydrazodicarbonamide, obtained by reaction of γ-isocyanofuran with anhydrous hydrazine in toluene, was suspended in 100 ml. of dry methylene chloride and oxidized with N-bromo-succinimide dissolved in pyridine at about -50°F (-45° C.). The reaction proceeded for 3-5 hours. The reaction product remained in solution and the unreacted hydrazo compound was removed by filtration. The filtrate was washed in succession with water, 2 percent hydrochloric acid, again water, 2 percent sodium bicarbonate solution, and again with water, in order to remove the reaction by products.

The structure for N,N'-di-(γ-furyl) azodicarbonamide was confirmed by infrared spectra analysis.

**EXAMPLE 22 - N,N'-BIS (2-TETRAHYDROFURFURYL)  
AZODICARBONAMIDE**



To 19.2 g of azodicarboxylic acid ethyl ester in 150 ml. of diethyl ether were added, at a temperature below 10°C., 20.2 g of tetrahydrofurfurylamine in 150 ml. of diethyl ether. An orange yellow solid amide separated out having a melting point of 100° - 104°C. By crystallization from ethyl acetate, orange red crystals having a melting point of 104°-107°C were obtained.

|           |    | Calculated | Found |
|-----------|----|------------|-------|
| Analysis: | C% | 50.65      | 50.73 |
|           | H% | 7.03       | 7.11  |
|           | N% | 19.70q     | 19.89 |

**EXAMPLE 23 - N,N' - DI - (γ -THIENYL)  
AZODICARBONAMIDE**

2.8 g of N,N'-γ-thienyl-hydrazodicarbonamide, obtained by reaction of γ-isocyanothiophene with anhydrous hydrazine in toluene was suspended in 100 ml. of dry methylene chloride and oxidized with N-bromo-succinimide dissolved in 20 ml. of pyridine at about -50°F (-45°C.).

The reaction proceeded for 3-4 hours. The reaction product remained in solution. The mass was filtered to remove the unreacted hydrazo compound, and the filtrate was washed in succession with water, 2 percent hydrochloric acid, again water, 2 percent sodium bicarbonate solution, and again with water. The structure for N,N'-di-(γ-thienyl) azodicarbonamide was confirmed by infrared spectra analysis.

**EXAMPLE 24 - N,N'-DIMORPHOLINO-  
AZODICARBONAMIDE**



5 17.5 (0.1 mol) of diethyl-azo-dicarboxylate dissolved in 100 ml. of ether were reacted at 41.0° to 50.0°F. (5° - 10°C.), with 17.4 g (0.2 mol) of morpholine dissolved in 100 ml. of ether. A reddish precipitate soon separated out, and the reaction was completed in about 20 additional minutes. The product was

10 suction filtered and was purified by crystallization from ethylacetate. Small, yellow-red needles melting at 275.0° - 278.6°F (135° - 137°C.) were obtained.

**EXAMPLE 25 - N,N' - BIS [2-(N-MORPHOLINO)ETHYL]-  
AZODICARBONAMIDE**



To 19.2 g of azodicarboxylic acid ethyl ester in 200 ml. of diethyl ether, at a temperature below 20°C., 25.2 g of N-2-aminoethyl-morpholine in 100 cc of diethyl ether were added. An orange crystalline solid amide separated out having a melting point of 143° - 150°C. By crystallization from propanol, orange red crystals having a melting point of 155° - 160°C were obtained.

|           |    | Calculated | Found |
|-----------|----|------------|-------|
| Analysis: | C% | 49.15      | 47.69 |
|           | H% | 7.61       | 7.53  |
|           | N% | 24.55      | 24.35 |

**EXAMPLE 26 - N,N' - DI - (N-PIPERIDINYL)-  
AZODICARBONAMIDE**



45 17.4 g (0.1 mol) of diethyl-azo-dicarboxylate dissolved in 100 ml. of ether were reacted 41.0° to 50.0 F. (5° - 10°C.) with 17.0 g (0.2 mol) of piperidine dissolved in 100 ml. of ether. The color of the solution changed from orange to red as the reaction proceeded. After 30 minutes the solution was concentrated to a volume of about 30 ml. Yellow-orange colored crystals were formed which exhibited a M.p. of 269.6° - 273.2°F (132° - 134°C.).

**EXAMPLE 27 - N,N' - DICYCLOHEXYL-  
AZODICARBONAMIDE**



To 17.4 g of azodicarboxylic acid ethyl ester in 100 ml. of diethyl ether, 19.85 g of cyclohexylamine in 150 ml. of diethyl ether, at a temperature lower than 10°C., were added. The reaction was isothermal and a yellow solid in form of powder separated out at once. The yellow solid washed with diethyl ether and a melting point of 187° - 190°C. By crystallization from ethanol, orange yellow needles having a melting point of 201° - 203°C were obtained.

|           |    | Calculated | Found |
|-----------|----|------------|-------|
| Analysis: | C% | 60.00      | 60.06 |
|           | H% | 8.54       | 8.66  |
|           | N% | 19.98      | 19.99 |

The compounds of the present invention are useful for inhibiting fog in silver chloride, silver bromide and silver iodide emulsions and in emulsions comprising mixtures of these silver halides (such as, for example, silver bromoiodide emulsions). The silver halide emulsions of the present invention may include various synthetic polymer substitutes or supplements for gelatin as colloidal binders, for example, dextran, polyvinylalcohol, polyvinylpyrrolidone, partially hydrolyzed polyvinylacetate, polyethylacrylate, polymethylmethacrylate, polyamides, and the like.

The emulsions of the present invention can be chemically sensitized by ripening with naturally active gelatin, by the addition of such chemical sensitizers as, for example, thiosulfate, allyl thiourea, thiocyanates, thiosulfanates, etc. Sensitization can additionally be carried out by the use of noble metal salts, (e.g., gold salts). The emulsions of the present invention may contain spectral sensitizers (e.g., cyanine and merocyanine dyes, etc.), couplers, surfactants, hardeners, stabilizers, antifoggants, plasticizers, anti-oxidizing agents, development accelerators, and in general may include any of the variety of various additives which commonly are used in the production of photographic silver halide emulsions. Any suitable support, such as polystyrene, polyester, cellulose acetate, polycarbonate, paper, glass, and the like, can be used for the photographic elements of the present invention. The azodicarbonamides of the present invention have been found especially effective in inhibiting the fog which commonly results from the use of a polyester (e.g., polyethylene terephthalate) support, or when unusually rapid processes for emulsion coating and drying are employed.

Incorporation of azodicarbonamides into silver halide emulsions is conveniently accomplished by adding the azodicarbonamides in solution to the emulsions at the time the emulsions are prepared. Although it is preferred to have the azodicarbonamide compounds incorporated into silver halide emulsion layers, fog and spot inhibition is obtained if the compounds are at least contacted with the silver halide as previously described. For example, fog-inhibiting amounts of the azodicarbonamide compounds may be placed in a layer adjacent a silver halide layer in a photographic element or may be employed in photographic processing solutions. The amounts of azodicarbonamide compound which may be effectively employed in a silver halide emulsion layer or in a layer or layers adjacent thereto may vary widely, and may be readily determined by routine experimentation. When employed in a silver halide photographic emulsion, it is preferred to use from 0.1 - 15 millimoles of azodicarbonamide compound per mole of silver.

The efficient fog-inhibiting capacity of compounds of the present invention may be more readily appreciated by reference to the following illustrative examples:

sensitometer and developed for 3 minutes at 68.0° F. (20° C.) in a developer having the following composition:

|   |                            |                  |
|---|----------------------------|------------------|
| 5 | Metol                      | 3 g.             |
|   | anhydrous sodium sulfide   | 50 g.            |
|   | hydroquinone               | 9 g.             |
|   | anhydrous sodium carbonate | 50 g.            |
|   | potassium bromide          | 3 g.             |
|   | water                      | to make 1000 ml. |

Test results in terms of fog and relative sensitivity are reported in Table 1 below for fresh emulsions and for emulsions stored for 15 days at 122.0° F. (50° C.) and 50 percent R.H.

TABLE 1

|    | Fresh                     | 15 days at 122.0° F.<br>(50° C. and 50%<br>R.H.) |      |                         |      |
|----|---------------------------|--------------------------------------------------|------|-------------------------|------|
|    |                           | Relative<br>sensitivity                          | Fog  | Relative<br>sensitivity | Fog  |
| 25 | Azodicarbonamide mM./MA.: |                                                  |      |                         |      |
| 0  |                           | 100                                              | 0.15 | 108                     | 0.24 |
| 1  |                           | 92                                               | 0.09 | 92                      | 0.17 |
| 3  |                           | 85                                               | 0.06 | 92                      | 0.10 |
| 10 |                           | 76                                               | 0.04 | 76                      | 0.08 |

## EXAMPLE 29

One portion of a silver bromoiodide emulsion layer containing 2 mole percent of AgI and 98 mole percent of AgBr on a cellulose triacetate support was overcoated with a protective layer 1.5  $\mu$  thick having the following composition:

|    |                            |                  |
|----|----------------------------|------------------|
| 40 | Gelatin                    | 15 g.            |
|    | 10% saponin-water solution | 5 ml.            |
|    | water                      | to make 1000 ml. |

45 A second portion of the emulsion layer was overcoated with a protective layer having the above composition which additionally contained 1 g of azodicarbonamide (added as a 0.5 g./100 cc. solution in dimethylformamide). The two portions were exposed and were subdivided into further portions which were developed in the developer of Example 28 for 3 and 10 minutes, respectively, at 68.0° F. (20° C.)

50 Test results are reported in the following Table 2:

TABLE 2

|                                     | Fresh | 15 days at 122.0° F. (50° C.)<br>and 50% R.H. |               |                |                         |               |                |
|-------------------------------------|-------|-----------------------------------------------|---------------|----------------|-------------------------|---------------|----------------|
|                                     |       | Relative<br>sensitivity                       | Fog<br>3 min. | Fog<br>10 min. | Relative<br>sensitivity | Fog<br>3 min. | Fog<br>10 min. |
| Control (no azodi-carbonamide)----- |       | 100                                           | 0.11          | 0.25           | 107                     | 0.14          | 0.28           |
| With azodicarbon-<br>amide-----     |       | 99                                            | 0.06          | 0.20           | 97                      | 0.11          | 0.22           |

## EXAMPLE 28

A high-sensitivity silver halide photographic emulsion containing 2.0 mole percent of AgI and 98 mole percent of AgBr was divided into four portions. One portion was spread, without further treatment, on a polyester support. Azodicarbonamide in dimethylformamide solvent (0.5 g./100 cc.) was added in the amounts set forth in Table 1 to the other emulsion portions which were then spread on polyester supports. The resulting photographic elements were then exposed in a

70 A high-sensitivity silver bromoiodide emulsion containing 1.5 mole percent of AgI and 98.5 mole percent of AgBr was divided into portions to which were added various selected compounds of the present invention in an amount of 1.5 millimoles/mole Ag. Development in the developer of Example 28 was carried out at 68.0° F. (20° C) for 3 and for 10 minutes, respectively.

The results are reported in the following Table 3:

## EXAMPLE 30

TABLE 3

| Compound of Example                                          | Fresh                |            |             | Aged 15 days, 50° C. 50% R.H. |            |             |
|--------------------------------------------------------------|----------------------|------------|-------------|-------------------------------|------------|-------------|
|                                                              | Relative sensitivity | Fog 3 min. | Fog 10 min. | Relative sensitivity          | Fog 3 min. | Fog 10 min. |
| Control                                                      | 100                  | 0.14       | 0.51        | 92                            | 0.20       | 0.60        |
| Azodicarbonamide (0.5 g./100 cc. dimethylformamide solution) | 78                   | 0.09       | 0.35        | 88                            | 0.15       | 0.33        |
| 1 (0.5 g./100 cc. ethanol solution)                          | 72                   | 0.06       | 0.30        | 82                            | 0.05       | 0.23        |
| 3 (0.5 g./100 cc. water solution)                            | 79                   | 0.08       | 0.31        | 86                            | 0.08       | 0.29        |
| 4 (0.5 g./100 cc. ethanol solution)                          | 80                   | 0.05       | 0.29        | 82                            | 0.06       | 0.28        |
| 5 (0.5 g./100 cc. water solution)                            | 90                   | 0.06       | 0.30        | 93                            | 0.08       | 0.28        |
| 6 (0.5 g./100 cc. water solution)                            | 87                   | 0.08       | 0.33        | 88                            | 0.10       | 0.30        |
| 7 (0.5 g./100 cc. ethanol solution)                          | 87                   | 0.12       | 0.41        | 94                            | 0.14       | 0.40        |
| 8 (0.5 g./100 cc. water solution)                            | 80                   | 0.08       | 0.29        | 89                            | 0.08       | 0.28        |
| 9 (0.5 g./100 cc. ethanol solution)                          | 37                   | 0.06       | 0.29        | 77                            | 0.05       | 0.31        |
| 12 (0.5 g./100 cc. water solution)                           | 90                   | 0.08       | 0.37        | 90                            | 0.08       | 0.43        |
| 13 (0.5 g./100 cc. water solution)                           | 90                   | 0.08       | 0.37        | 90                            | 0.08       | 0.43        |

## EXAMPLE 31

To portions of an emulsion containing 1.75 mole percent of AgI and 98.25 mole percent of AgBr were added azodicarbonamide and N,N'-diethyl-azodicarbonamide. Sensitivity and fog were measured for both fresh samples and samples which has been aged for 15 days at 122.0° F. (50° C.) and at 50 percent R.H.

The results are summarized in the following Table 4.

TABLE 4

| Compound                                                       | Fresh      |                      |      | Aged 15 days at 50° C. and 50% R.H. |      |
|----------------------------------------------------------------|------------|----------------------|------|-------------------------------------|------|
|                                                                | mM./M. Ag. | Relative sensitivity | Fog  | Relative sensitivity                | Fog  |
| Control                                                        |            | 100                  | 0.24 | 100                                 | 0.43 |
| Azodicarbonamide (0.5 g./100 cc. dimethylformamide solution)   | 0.3        | 100                  | 0.23 | 100                                 | 0.28 |
| Do                                                             | 0.5        | 90                   | 0.22 | 110                                 | 0.28 |
| Do                                                             | 0.6        | 90                   | 0.21 | 110                                 | 0.28 |
| N,N'-diethylazodicarbonamide (0.5 g./100 cc. ethanol solution) | 0.3        | 110                  | 0.20 | 110                                 | 0.36 |
| Do                                                             | 0.6        | 100                  | 0.20 | 110                                 | 0.32 |
| Do                                                             | 0.9        | 100                  | 0.19 | 100                                 | 0.32 |

## EXAMPLE 32

To illustrate the inhibiting effect exerted by the subject <sup>40</sup> and 30 percent R.H. are reported in Table 6.

TABLE 6

| Compound of Example                   | mM./M. Ag. | Relative sensitivity, fresh | Relative sensitivity, aged | Fog, fresh | Fog, aged |
|---------------------------------------|------------|-----------------------------|----------------------------|------------|-----------|
| Control                               |            | 100                         | 100                        | 0.52       | 0.60      |
| 14 (0.5 g./100 cc. ethanol solution)  | 0.5        | 99                          | 104                        | 0.33       | 0.37      |
| 15 (0.5 g./100 cc. ethanol solution)  | 0.5        | 102                         | 103                        | 0.39       | 0.41      |
| 16 (0.5 g./100 cc. ethanol solution)  | 0.5        | 102                         | 103                        | 0.37       | 0.44      |
| 17 (0.25 g./100 cc. ethanol solution) | 0.15       | 100                         | 103                        | 0.34       | 0.46      |

compounds on the formation of spots caused by the presence of metal particles, the following test was performed:

A high-sensitivity emulsion chemically ripened with gold thiosulfate and thiocyanate was divided in two portions A (control) and B. 0.5 millimoles of azodicarbonamide (0.5 g./100 cc dimethylformamide solution/mole Ag) were added to part B. The two emulsions were spread on a polyester support which had previously been dusted with fine iron powder. After drying and without exposure, the two portions were developed as described in example 28. The ability of the compound to inhibit the formation of black and white spots was determined by counting the number of spots per unit area for three samples of each of the portions A and B.

The results are reported in the following Table 5.

TABLE 5

|                                                | 1st sample | 2nd sample | 3rd sample |
|------------------------------------------------|------------|------------|------------|
| A (control)                                    | 52         | 47         | 80         |
| B (0.5 millimoles of azodicarbonamide/mole Ag) | 5          | 1          | 3          |

## EXAMPLE 33

A silver halide photographic emulsion containing 98 mole

percent of AgBr and 2 mole percent of AgI was divided into several portions. One portion (control) was spread on a polyester support without further treatment. The other emulsion portions were coated on identical polyester supports after adding thereto solutions of selected representative compounds of the present invention. The resulting photographic elements were then exposed in a sensitometer and developed for 90 seconds in the developer of Example 28. The results of

20

sensitometric tests carried out, respectively, on fresh emulsions and on emulsions aged for 15 hours at 161.6° F. (72° C.)

40

and 30 percent R.H. are reported in Table 6.

## EXAMPLE 34

To portions of a silver halide photographic emulsion containing 1.5 mole percent of AgI and 98.5 mole percent of AgBr were added selected compounds of the present invention in the amounts and solvents given in Table 7. Each portion was then coated on a polyester support which had been pre-coated with a subbing layer of gelatin containing iron powder suspended therein. The resulting photographic elements were maintained in a cooled condition for 10 minutes before drying, and were subsequently processed for 90 seconds in the developer of Example 28. Thereafter the black sensitization spots caused by the presence of the iron particles were counted. The results are reported in Table 7.

55

60

65

TABLE 7

| Compound of Example: | mM./M. Ag | Subbing layer with iron powder | Number of black spots per 70 sq. cm. |
|----------------------|-----------|--------------------------------|--------------------------------------|
| 14                   | 0.5       | do                             | 2                                    |
| 14                   | 1.0       | do                             | 53                                   |
| 15                   | 0.5       | do                             | 3                                    |
| 15                   | 1.0       | do                             | 180                                  |
| 16                   | 0.5       | do                             | 117                                  |
| 16                   | 1.0       | do                             | 10                                   |
| 16                   | 1.0       | do                             | 0                                    |
| 17                   | 0.15      | do                             | 55                                   |
| 17                   | 0.5       | do                             | 6                                    |

## EXAMPLE 35

A silver halide photographic emulsion containing 98 mole percent of AgBr and 2 percent of AgI, and characterized by a high silver to gelatin ratio, was divided into several parts. One of these was spread and cellulose triacetate without further additions. The other parts were spread after adding thereto solutions (0.5 g./100 cc. 1/20 N H<sub>2</sub>SO<sub>4</sub>) of the compounds of Examples 18 and 19 in varying amounts. Samples of the emulsions were then exposed in a sensitometer and tray-developed for five minutes at 68.0° F. (20° C.) in the developer of Example 28. Table 8 reports the results of sensitometric tests carried out on fresh emulsions and on emulsions which had been aged for 15 hours at 72° C. and 30 percent R.H.

TABLE 8

| Compound of Example | Mm./M.Ag | Relative sensitivity (aged; 15h; 30% R.H. 161.6° F. (72° C.)) |           | Fog (aged; 15h; 30% R.H. 161.6° F. (72° C.)) |                               |
|---------------------|----------|---------------------------------------------------------------|-----------|----------------------------------------------|-------------------------------|
|                     |          | Relative sensitivity, fresh                                   | (72° C.)) | Fog, R.H. 161.6° F. (72° C.))                | Fog, R.H. 161.6° F. (72° C.)) |
| Control             |          | 100                                                           | 100       | 0.31                                         | 0.32                          |
| 18                  | 0.1      | 100                                                           | 100       | 0.31                                         | 0.32                          |
| 18                  | 0.5      | 95                                                            | 80        | 0.25                                         | 0.28                          |
| 18                  | 2.5      | 76                                                            | 67        | 0.19                                         | 0.19                          |
| 19                  | 0.1      | 95                                                            | 80        | 0.31                                         | 0.31                          |
| 19                  | 0.5      | 80                                                            | 80        | 0.20                                         | 0.20                          |

EXAMPLE 36

Example 35 was repeated with portions of a similar emulsion which contained 98 mole percent AgBr and 2.0 mole percent AgI and to which the compounds of Examples 21 and 23 had been added. Results are reported in Table 9.

TABLE 9

| Compound of Example                   | Mm./M.Ag | Relative sensitivity (aged; 15 h; 30% R.H. 161.6° F. (72° C.)) |           | Fog (aged; 15h; 30% R.H. 161.6° F. (72° C.)) |                               |
|---------------------------------------|----------|----------------------------------------------------------------|-----------|----------------------------------------------|-------------------------------|
|                                       |          | Relative sensitivity, fresh                                    | (72° C.)) | Fog, R.H. 161.6° F. (72° C.))                | Fog, R.H. 161.6° F. (72° C.)) |
| Control                               |          | 100                                                            | 100       | 0.50                                         | 0.57                          |
| 21 (0.5 g./100 cc. ethanol solution)  | 0.1      | 80                                                             | 110       | 0.30                                         | 0.35                          |
| 21 (0.5 g./100 cc. ethanol solution)  | 0.5      | 63                                                             | 97        | 0.26                                         | 0.32                          |
| 23 (1.0 g./100 cc. pyridine solution) | 0.05     | 70                                                             | 80        | 0.36                                         | 0.38                          |
| 23 (1.0 g./100 cc. pyridine solution) | 0.1      | 50                                                             | 68        | 0.31                                         | 0.33                          |

EXAMPLE 37

Example 35 was repeated with a similar emulsion which contained 98 mole percent AgBr and 2.0 mole percent AgI and to which the compounds of Examples 24 and 26 had been added. Results are reported in Table 10.

55

EXAMPLE 39

Example 35 was duplicated except that solutions of the compounds of Examples 10, 11, 22, 25 and 27 were employed. Each compound was dissolved in ethanol at a concentration of 0.5 g./100 cc. Results are reported in Table 12.

TABLE 10

| Compound of Example                   | Mm./M.Ag | Relative sensitivity (aged; 15 h; 30% R.H. 161.6° F. (72° C.)) |           | Fog (aged; 15h; 30% R.H. 161.6° F. (72° C.)) |                               |
|---------------------------------------|----------|----------------------------------------------------------------|-----------|----------------------------------------------|-------------------------------|
|                                       |          | Relative sensitivity, fresh                                    | (72° C.)) | Fog, R.H. 161.6° F. (72° C.))                | Fog, R.H. 161.6° F. (72° C.)) |
| Control                               |          | 100                                                            | 100       | 0.25                                         | 0.28                          |
| 24 (0.5 g./100 cc. ethanol solution)  | 0.1      | 107                                                            | 105       | 0.25                                         | 0.26                          |
| 24 (0.5 g./100 cc. ethanol solution)  | 0.5      | 93                                                             | 105       | 0.16                                         | 0.16                          |
| 24 (0.5 g./100 cc. ethanol solution)  | 2.5      | 57                                                             | 61        | 0.09                                         | 0.09                          |
| 26 (1.0 g./100 cc. pyridine solution) | 0.1      | 100                                                            | 100       | 0.23                                         | 0.24                          |
| 26 (0.1 g./100 cc. pyridine solution) | 0.5      | 96                                                             | 105       | 0.20                                         | 0.19                          |
| 26 (1.0 g./100 cc. pyridine solution) | 2.5      | 74                                                             | 76        | 0.10                                         | 0.13                          |

TABLE 12

| Compound of Example | mM/M Ag | Fresh                |      | Stored: 15h; 30% R.H. 72° C. |      |
|---------------------|---------|----------------------|------|------------------------------|------|
|                     |         | Relative sensitivity | Fog  | Relative sensitivity         | Fog  |
| Control             |         | 100                  | 0.31 | 100                          | 0.32 |
| 10                  | 0.0125  | 79                   | 0.17 | 81                           | 0.20 |
| 11                  | 0.025   | 79                   | 0.29 | 85                           | 0.28 |
|                     | 0.050   | 79                   | 0.18 | 85                           | 0.17 |
| 22                  | 0.10    | 95                   | 0.28 | 96                           | 0.30 |
|                     | 0.50    | 95                   | 0.20 | 96                           | 0.20 |
|                     | 2.50    | 68                   | 0.11 | 68                           | 0.11 |
| 25                  | 0.5     | 89                   | 0.18 | 69                           | 0.20 |
| 27                  | 0.10    | 100                  | 0.22 | 89                           | 0.30 |
|                     | 0.50    | 79                   | 0.19 | 89                           | 0.18 |

What is claimed is:

1. A silver halide photographic emulsion having contacted therewith as a fog-inhibitor an azodicarbonamide.

2. The emulsion of claim 1 having from about 0.1 to 15 millimoles of said compound per mole of silver in said silver halide.

3. A silver halide photographic emulsion having contacted therewith as a fog-inhibitor a compound of the formula



wherein  $\text{R}_1$ ,  $\text{R}_2$ ,  $\text{R}_3$  and  $\text{R}_4$  individually are hydrogen or an alkyl, aryl or heterocyclic group or wherein the pairs of groups  $\text{R}_1 - \text{R}_2$  or  $\text{R}_3 - \text{R}_4$  represent atoms necessary to complete a heterocyclic ring.

4. A photographic element comprising a silver halide emulsion layer and, in fog-inhibiting association therewith, a fog-inhibitor of the formula



5. wherein  $\text{R}_1$ ,  $\text{R}_2$ ,  $\text{R}_3$  and  $\text{R}_4$  individually are hydrogen or an alkyl, aryl or heterocyclic group or wherein the pairs of groups  $\text{R}_1 - \text{R}_2$  or  $\text{R}_3 - \text{R}_4$  represent atoms necessary to complete a heterocyclic ring.

10. The photographic element of claim 4 wherein said fog-inhibitor is contained in a layer adjacent said silver halide emulsion layer.

11. The photographic element of claim 4 wherein said fog-inhibitor is incorporated within said emulsion layer.

12. The photographic element of claim 6 wherein said emulsion layer contains from about 0.1 to about 15 millimoles of said fog-inhibitor per mole of silver in said silver halide.

13. A photographic element comprising a silver halide emulsion layer and, in fog-inhibiting association therewith, an azodicarbonamide as a fog-inhibitor.

14. An azodicarbonamide fog-inhibitor of the formula



25. wherein  $\text{R}_5$ ,  $\text{R}_6$ ,  $\text{R}_7$  and  $\text{R}_8$  may be hydrogen and wherein at least one of  $\text{R}_5$ ,  $\text{R}_6$ ,  $\text{R}_7$  and  $\text{R}_8$  is an alkoxyalkyl, alkoxyaryl, hydroxyalkyl, haloaryl, allyl, heterocyclic or heterocyclic-alkyl group.

30. 10. A photographic element comprising a polyester support, a silver halide emulsion layer and, in fog-inhibiting association with said silver halide emulsion layer, an azodicarbonamide as a fog-inhibitor.

35. 11. A method for inhibiting fog in a silver halide emulsion comprising contacting said emulsion with an azodicarbonamide compound.

\* \* \* \* \*

40

45

50

55

60

65

70

75

UNITED STATES PATENT OFFICE  
CERTIFICATE OF CORRECTION

Patent No. 3,655,391

Dated April 11, 1972

Inventor(s) Paoli Merli and Luigi Valbusa

It is certified that error appears in the above-identified patent and that said Letters Patent are hereby corrected as shown below:

Page 1, after the heading "Inventors" and before the heading "Filed", insert -- Assignee: Minnesota Mining and Manufacturing Company, St. Paul, Minnesota --;

Column 4, line 56, "164-162°C." should be -- 164-165°C. --;

Column 8, line 18, formula of Example 25,



Signed and sealed this 28th day of November 1972.

(SEAL)  
Attest:

EDWARD M.FLETCHER, JR.  
Attesting Officer

ROBERT GOTTSCHALK  
Commissioner of Paten